

## 1

3,551,214  
**COPPER ALLOY EXHIBITING GAMMA ALUMINA SURFACE AND METHOD**  
James A. Ford, North Haven, Elmer J. Caule, New Haven, and Philip R. Sperry, North Haven, Conn., assignors to Olin Corporation, a corporation of Virginia  
No Drawing. Filed Jan. 29, 1968, Ser. No. 701,062  
Int. Cl. C23f 7/02; C22c 9/00  
U.S. Cl. 148—6.31      14 Claims

### ABSTRACT OF THE DISCLOSURE

A tarnish resistant alloy consisting essentially of from 1.0 to 9.5% aluminum, up to 5.5% silicon, 0.01 to 0.5% of either phosphorus, arsenic, selenium and bismuth, and at least one element from the group of from 0.05 to 1.5% zinc, 0.05 to 0.3% cadmium, 0.05 to 0.3% beryllium, and 0.05 to 0.5% magnesium, balance copper, and the method of producing the alloy.

### DISCLOSURE

It has been disclosed in U.S. Pat. No. 3,259,491 that proper combinations of ternary alloying additions to Cu, which were selected on the basis of being capable of forming a complex stable oxide, of having sufficient solid solubility in Cu to be available for diffusion under proper conditions to the metal surface and being balanced to provide diffusion to the surface in proper proportions to form the stable oxide, will provide unusual oxidation resistance.

It has further been shown in U.S. Pat. 3,341,369 that the class of copper base alloys containing combinations of Group III with Group IV alloying additions, not only show good elevated temperature oxidation resistance, but also provide enhanced oxidation resistance at lower temperatures in the metal surface beneath the original continuous oxide film. These alloys when heated in an oxidizing atmosphere at high temperatures, e.g. 750° C., form a transparent oxide film which both preserves the original color and luster of the alloy, and also provides the oxidation and improved tarnish resistance.

Also, in U.S. application S.N. 584,097, filed Oct. 4, 1966, Group V elements including phosphorus, arsenic, antimony, and bismuth have been found desirable for enhanced tarnish resistance in the alumina film formed at elevated temperature, e.g. 450° C. to 800° C.

As is also disclosed in said Ser. No. 584,097, the previously mentioned Group V elements are equally effective in an alloy containing cobalt containing 0.05 to 5% cobalt, e.g. Cu—3Al—2Si—0.1P—0.3Co.

Although these alloys do afford excellent oxidation resistance at elevated temperatures, they do not form protective films at lower temperatures down to, and including, ambient.

It is an object of the present invention to extend the range of temperature toward ambient over which a highly protective oxide film is formed.

It is another object of the present invention to provide a tarnish resistant alloy.

The protective oxide film formed on the foregoing alloys has been identified as gamma alumina. It is known

## 2

that gamma alumina has a defect spinel structure and that suitable alloying will provide changes in its resistance to ionic movement under a potential. Experience gained with additions to Al alloys has demonstrated that, for example, a small addition of Mg (0.1%) will increase both the ionic and electronic resistance of the alumina film and limit its growth. However, larger additions reverse this behavior by promoting the formation of MgO, rather than alumina.

Based on these considerations, the present invention embodies additions which, when present in the alloy solid solution in small amounts, will promote the formation of more perfect oxide films, with resulting enhanced oxidation and tarnish resistance. In the same sense that small amounts of specific impurities added to semi-conducting compounds will have large effects on their conductive properties, these minor additions can be considered as "dopants" for the oxide formed on the metal surface.

In order to achieve the desired improved oxide film, specifically an alumina film on the Cu—Al—Si Group V alloy, small additions of Group II elements Zn, Cd, Be and Mg have been made. The Group II additions may be provided in the following compositional ranges to the basic alloy:

|    | Percent  |
|----|----------|
| Zn | 0.05—1.5 |
| Cd | 0.05—0.3 |
| Be | 0.05—0.3 |
| Mg | 0.05—0.5 |

It has been found that the most favorable alloying combination with the Group II elements is 1.0 to 9.5% Al, and up to 5.5% Si. Furthermore, the optimum alloy composition has been established at 2 to 4% Al and 1 to 3% Si.

It has also been found that the previously mentioned Group V elements (P, As, Sb, Bi) can be used in combination with the Group II elements in the range of 0.01 to 0.5%. However, the preferred Group V element is phosphorous.

Cobalt also may be used in the range of 0.05 to 5%. These alloys may be thermally oxidized over the temperature range of 300°—550° C., from 5 minutes to 100 hours in an oxidizing atmosphere. Even longer oxidizing times could be utilized, if desired, but in general are not justifiable economically.

The following examples illustrate the invention without limiting its scope.

### EXAMPLES

The table below contains data obtained from oxidizing copper base alloys containing 3% aluminum, 2% silicon, and 0.1% phosphorus at various temperatures. The particular alloy additions are given in the left-hand column. At each of the temperatures specified, the alloys were oxidized for a period of time of two hours. A capacitance bridge technique was used for measuring the film resistance reported. See, for example, Beck et al., International Journal of Corrosion Science, vol. 2, pp. 133—145, 1962.

The results in the table show that the cadmium, beryllium, zinc, and magnesium all provide tarnish resistance after exposure to the outdoors (roof exposure racks) for respectively, 10 and 70 days, provided that the alloys are oxidized within a temperature range of from 350 to 550° C.

## IONIC RESISTANCE OF FILM ON DOPED MRL-B2 (CU-3AL-2SH-0.1P) FORMED AT VARIOUS TEMPERATURES COMPARED WITH OUTDOOR TARNISH RESISTANCE

| Alloy No. | Donant and amount, w/o | 25° C.             |                                       |                        | 35° C.             |                                       |                        | 45° C.             |                                       |                        | 55° C.             |                                       |                        |
|-----------|------------------------|--------------------|---------------------------------------|------------------------|--------------------|---------------------------------------|------------------------|--------------------|---------------------------------------|------------------------|--------------------|---------------------------------------|------------------------|
|           |                        | Film thickness, A. | Film resistance, ohm-cm. <sup>2</sup> | Film behavior, 70 days | Film thickness, A. | Film resistance, ohm-cm. <sup>2</sup> | Film behavior, 70 days | Film thickness, A. | Film resistance, ohm-cm. <sup>2</sup> | Film behavior, 70 days | Film thickness, A. | Film resistance, ohm-cm. <sup>2</sup> | Film behavior, 70 days |
| 668.....  | 0.1Zn.....             | 30                 | 1,378                                 | Poor.....              | 42                 | 2,222                                 | Poor.....              | 86                 | 4,317                                 | Poor.....              | 143                | 23,955                                | Good.....              |
| 669.....  | 0.5Zn.....             | 18                 | 264                                   | Poor.....              | 41                 | 2,247                                 | Poor.....              | 76                 | 3,973                                 | Poor.....              | 167                | 24,479                                | Good.....              |
| 670.....  | 1.0Zn.....             | 21                 | 499                                   | Poor.....              | 43                 | 2,409                                 | Poor.....              | 82                 | 2,911                                 | Poor.....              | 154                | 18,661                                | Fair(2).....           |
| 671.....  | 2.0Zn.....             | 16                 | 316                                   | Poor.....              | 35                 | 1,751                                 | Poor.....              | 84                 | 7,216                                 | Poor.....              | 146                | 21,333                                | Good.....              |
| 672.....  | 0.5Zn + 0.3Co.....     | 21                 | 606                                   | Poor.....              | 39                 | 1,294                                 | Poor.....              | 87                 | 4,970                                 | Poor.....              | 130                | 4,886                                 | Poor.....              |
| 673.....  | 0.1Be.....             | 15                 | 166                                   | Poor.....              | 69                 | 2,747                                 | Poor.....              | 107                | 9,870                                 | Poor.....              | 169                | 21,111                                | Good.....              |
| 674.....  | 0.2Be.....             | 18                 | 236                                   | Poor.....              | 61                 | 4,970                                 | Fair(2).....           | 114                | 12,018                                | Poor.....              | 223                | 16,688                                | Fair(1).....           |
| 675.....  | 0.3Be.....             | 21                 | 551                                   | Poor.....              | 64                 | 1,609                                 | Fair(2).....           | 118                | 14,054                                | Poor.....              | 279                | 37,932                                | Good.....              |
| 676.....  | 0.1Mg.....             | 18                 | 203                                   | Poor.....              | 32                 | 533                                   | Poor.....              | 56                 | 1,419                                 | Fair(2).....           | 63                 | 1,419                                 | Fair.....              |
| 677.....  | 0.5Mg.....             | 16                 | 227                                   | Poor.....              | 19                 | 219                                   | Poor.....              | 10                 | 1,95                                  | Poor.....              | 10                 | 1,95                                  | Poor.....              |
| 678.....  | 0.1Co.....             | 30                 | 960                                   | Poor(1)....            | 43                 | 2,601                                 | Fair(1)....            | 96                 | 13,463                                | Good(1)....            | 149                | 17,827                                | Fair(2).....           |
| 679.....  | 0.3Cd.....             | 25                 | 604                                   | Poor.....              | 41                 | 887                                   | Fair(2)....            | 83                 | 7,112                                 | Poor.....              | 143                | 20,546                                | Good.....              |
| 680.....  | 0.5Cd.....             | 21                 | 400                                   | Poor.....              | 47                 | 2,200                                 | .....                  | 77                 | 5,000                                 | .....                  | 146                | 16,000                                | .....                  |

<sup>1</sup> Cu-3Al-2Sh-0.3Co-0.1P (for comparison only—not exposed).

Note: Numbers in parentheses represent standing among specimens based on appearance at the particular exposure time for a given heat treat temperature.

It is to be understood that the invention is not limited to the illustrations described and shown herein, which are deemed to be merely illustrative of the best modes of carrying out the invention and which are susceptible of modifications of form, size, arrangement of parts and detail of operation. The invention rather is intended to encompass all such modifications which are within the spirit and scope of the invention as set forth in the appended claims.

10 What is claimed is:

1. A copper base alloy having improved tarnish resistance consisting essentially of:

15 1.0 to 9.5% aluminum,

up to 5.5% silicon,

0.01 to 0.5% of a Group V element selected from the group consisting of P, As, Se, and Bi, and

at least one element selected from the group consisting of.

20 Zn 0.05 to 1.5%

Cd 0.05 to 0.3%

Be 0.05 to 0.3%, and

Mg 0.05 to 0.5%

25 said alloy having a tarnish resistant gamma alumina film on the surface thereof.

2. An alloy according to claim 1 which contains approximately 2 to 4% aluminum, 1 to 3% silicon, and approximately 0.1% phosphorus.

3. An alloy according to claim 2 also containing from 0.05 to 5% cobalt.

4. An alloy according to claim 3 containing approximately 0.3% cobalt.

5. An alloy according to claim 1 containing 0.05 to 0.3% Cd.

6. An alloy according to claim 1 containing 0.05 to 0.3% Be.

7. An alloy according to claim 1 containing .05 to 0.5% Mg.

8. A process for providing a copper base alloy having improved tarnish resistance comprising providing an alloy consisting essentially of:

45 1.0 to 9.5% aluminum

up to 5.5% silicon

0.01 to 0.5% of at least one Group V element selected from the group consisting of P, As, Se, and Bi,

50 and at least one element selected from the group consisting of:

Zn 0.05 to 1.5%

Cd 0.05 to 0.3%

Be 0.05 to 0.3%

Mg 0.05 to 0.5%, and

oxidizing said alloy at a temperature of from 300° to 550° C. for at least five minutes in order to form a tarnish resistant gamma alumina film on the surface thereof.

60 9. A process according to claim 8 in which the copper base alloy contains approximately 2 to 4% aluminum, 1 to 3% silicon, and approximately 0.1% phosphorus.

10. A process according to claim 8 in which the alloy contains from 0.05 to 5% cobalt.

11. A process according to claim 8 in which the temperature is 350 to 550° C.

12. A process according to claim 8 in which said one element is Cd in the range of 0.05 to 0.3%.

70 13. A process according to claim 8 in which said one element is Be in the range of 0.05 to 0.3%.

14. A process according to claim 8 in which said one element is Mg in the range of 0.05 to 0.5%.

**5****References Cited****UNITED STATES PATENTS**

|           |         |               |         |
|-----------|---------|---------------|---------|
| 2,093,380 | 9/1937  | Morris        | 75—162  |
| 2,130,737 | 9/1938  | Hensel et al. | 75—162X |
| 3,259,491 | 7/1966  | Pryor         | 75—162  |
| 3,475,227 | 10/1969 | Capula et al. | 75—153X |

**6****FOREIGN PATENTS**

|                                     |      |               |        |
|-------------------------------------|------|---------------|--------|
| 138,568                             | 1934 | Austria       | 75—162 |
| 519,902                             | 1940 | Great Britain | 75—162 |
| CHARLES N. LOVELL, Primary Examiner |      |               |        |
| U.S. Cl. X.R.                       |      |               |        |
| 75—153, 157.5, 160, 162; 148—31.5   |      |               |        |

5